

Sept. 4, 1951

A. F. GRUPP ET AL  
PRESSURE SENSITIVE DECALCOMANIA  
AND METHOD OF MAKING THE SAME  
Filed Nov. 29, 1947

2,567,067

*Fig. 1.*



*Fig. 2.*



*Fig. 3.*



*Fig. 4.*



*Fig. 5.*



Inventors:-  
Alfred F. Grupp,  
Harry C. Rathke,  
Elwood S. Tolan,  
Elmore Watts,

*By Davis, Lindsey, Kitten & Rogers Atty's.*

## UNITED STATES PATENT OFFICE

2,567,067

PRESSURE SENSITIVE DECALCOMANIA AND  
METHOD OF MAKING THE SAME

Alfred F. Grupp, Glen Ellyn, Harry C. Rathke and  
Elwood S. Talan, Chicago, Ill., and Elmore  
Watts, Mission, Kans., assignors to The Meyer-  
cord Co., Chicago, Ill., a corporation of Illinois

Application November 29, 1947, Serial No. 788,816

16 Claims. (Cl. 117—3.6)

1

This invention relates to a novel transfer of the decalcomania type and to a method of manufacturing the same.

Heretofore, pressure sensitive decalcomanias have been produced and used with varying degrees of success. Generally, in the use of such decalcomanias, a paper backing is removed from the decalcomania in the usual manner by soaking in water thereby exposing a tacky, pressure sensitive, adhesive layer which may be applied directly to the surface to be decorated. Upon the application of pressure, the transfer is caused to adhere to the surface.

Pressure sensitivity has long been recognized as a desirable property in a decalcomania since it provides a quick, effective, and simple means for applying the transfer without the necessity of using solvents and special adhesives. However, numerous difficulties and disadvantages have been encountered and they have made it impossible heretofore to produce a satisfactory pressure sensitive decalcomania in a quick, inexpensive, and simple manner. For example, the pressure sensitive adhesives, which remain tacky during production and over an extended portion of the life of the decalcomania, are not directly printable and normally require the application of a sealer coating over the adhesive layer in order to overcome the tackiness and to provide a firm, non-tacky surface capable of receiving an imprint without running and without adhering to the printing rolls or screens. Moreover, during the manufacturing process, the resultant wet transfer sheets possess a high degree of tack and consequently are not stackable necessitating the provision of elaborate and bulky drying racks to permit the individual decalcomania sheets to be stored out of contact with each other until application of the sealer coating.

Another disadvantage possessed by the known types of pressure sensitive decalcomanias is that the adhesive tends to remain in a normally tacky condition for some period of time after application to a surface thereby permitting the decalcomanias to be removed without destruction thereof. Such ease of removal is highly undesirable particularly where it is necessary to guard against theft and re-use. It has also been found that the pressure sensitivity and normal tackiness of such adhesive layers finally disappear and the adhesive becomes dry and cracks after a considerable period of time with the result that the decalcomania becomes loosened and often falls from the surface to which it has been originally applied.

2

One object of the present invention is to provide a novel decalcomania transfer which has pressure sensitive properties in the adhesive layer but which is not subject to the many disadvantages and difficulties previously associated with the production of a pressure sensitive type decalcomania.

Another object of the invention is to provide a decalcomania which has pressure sensitive properties and yet is readily stackable during its manufacture, particularly after the application of the adhesive layer.

Another object of the invention is to provide a decalcomania having pressure sensitive properties but which does not require the use of a sealer layer.

Still another object is to provide a decalcomania of the pressure sensitive type in which the adhesive layer, after being applied to the carrier paper, quickly dries to a substantially dry, non-tacky, and non-pressure sensitive adhesive thereby permitting the sheets to be stacked during production without adhering to each other while awaiting application of the design prints, the adhesive layer, however, being of such properties as to become pressure sensitive and tacky upon application of additional layers thereover.

A still further object of the invention is to provide a novel decalcomania which possesses pressure sensitive properties serving to provide a preliminary adhesive bond for holding the decalcomania in place when first applied to a surface and which, with the passage of time, develops a permanent, tough, strong, scratch resistant, adhesive bond with said surface.

An additional object of the invention is to provide a novel decalcomania of the pressure sensitive type in which the degree of tack or pressure sensitivity of the adhesive may be controlled or varied in accordance with the uses to which the decalcomania is to be put and thereby adapting it for application to a wide variety of rough, porous, plastic, or metallic surfaces.

Another object of the invention is to provide a novel decalcomania in which the adhesive stratum as initially applied is normally non-tacky and non-pressure sensitive but which, after the application of subsequent layers, is converted by the action of plasticizing oils in said subsequent layers to a tacky, pressure sensitive stratum.

A decalcomania transfer consists ordinarily of a relatively heavy absorbent type paper backing coated with a water soluble adhesive or gum to which are applied a plurality of additional strata or films such as a water insoluble adhesive layer,

a transfer design in color, and a protective coating. The decalcomania of the present invention differs from the decalcomanias previously known by the provision of a plurality of independent but interacting layers of which one layer comprises a resinous, normally non-pressure sensitive material and of which at least one other layer contains one or more plasticizers capable of migrating or diffusing into the resinous layer to convert the latter into a tacky, pressure sensitive adhesive. Inasmuch as the potential pressure sensitivity of the adhesive layer does not develop until after migration of the plasticizing oils has occurred, it will be apparent that our decalcomania is based upon what may be characterized as a "delayed action" principle, and as a result we are able to avoid the printing and stacking difficulties previously encountered in the production of a pressure sensitive decalcomania.

The major component of the adhesive layer of our decalcomania is a thermoplastic, water insoluble, non-oxidizing resin which is normally non-tacky and non-pressure sensitive but which is capable of being converted by the action of a suitable plasticizer to a tacky, pressure sensitive condition. The adhesive stratum is applied in the form of a solution of the resin in a suitable quick-drying solvent or vehicle. After evaporation of the solvent which occurs after the lapse of a very short time, the dry adhesive layer is non-tacky and non-pressure sensitive and may be stacked or printed upon in the customary manner without difficulty. In one embodiment of the invention an activating lacquer or coating containing an appropriate and predetermined amount of plasticizer for the resin may be applied preferably directly over the adhesive layer, although the juxtaposition of the adhesive and activating strata is not essential, and after a suitable period of time has elapsed, the plasticizing oils will have migrated or diffused into the adhesive layer converting the resinous constituent thereof to a tacky, pressure sensitive material. In other embodiments of the invention no special activating layer is employed, but the normal plasticizer content of the various layers of printing lacquers forming the transfer design is sufficient to migrate into the resinous adhesive layer and render it tacky. The plasticizing oils thus serve to create tackiness in the adhesive layer as well as to maintain the lacquers in a flexible state but the tackiness of the adhesive layer does not in any way prevent the activating lacquer or the printing lacquers from drying to a non-tacky state. By varying the resin content of the adhesive layer, the thickness of the layer, and the amount and character of the plasticizer in the activating and later printed layers, the degree of tackiness or pressure sensitivity may be controlled within definite limits.

The mechanism and structure of the decalcomanias of the present invention will become more apparent by reference to the drawing wherein several alternative arrangements embodying the migration principle are illustrated in cross-section with the various strata or films shown in exaggerated thickness for the sake of clarity. Similar reference characters are employed to designate corresponding strata throughout the several views, the letter B referring generally to a paper backing, D to a water soluble gum such as dextrose, R to a water insoluble, resinous adhesive layer which is originally non-pressure sensitive but later assumes pressure sensitive characteristics, A to an activating coating containing

plasticizing oils, P to color printing layers, C to a clear lacquer protective coating, and S to a sealer coating.

Figure 1 is a cross-section of one form of decalcomania embodying the present invention and showing a special activating layer superimposed directly over the resinous adhesive layer.

Fig. 2 is an alternative form of decalcomania comprising the present invention in which the activating coat is separated from the adhesive layer by means of an intervening printed layer.

Fig. 3 illustrates a third form of the invention.

Fig. 5 shows a "reverse" type decalcomania in which the activating coat is applied over the color printing layer and the adhesive layer is superimposed directly over the activating coat.

Fig. 4 is still another embodiment of the invention in which no special activating layer is employed and in which the migratory plasticizing oils are supplied in the layers of printing lacquer applied over the resinous adhesive layer.

Fig. 5 shows a "reserve" type decalcomania in which the resinous adhesive layer is applied directly over the printing layer and no special activating layer is employed.

Referring to the form of decalcomania shown in Fig. 1, the layer B is a paper backing or carrier of the absorbent type well known to the decalcomania art. This paper is surfaced with a layer D of a water soluble adhesive or gum such as dextrose, gelatine, gum tragacanth, etc. which, upon wetting with water, will permit the paper base or backing to be removed from the transfer.

Over the layer D is applied by printing or screening in the usual manner a film R of a thermoplastic, non-oxidizing, water insoluble, normally non-tacky and non-pressure sensitive resin in solution in a suitable quick-drying solvent. The resins which may be employed in the adhesive layer R may be of a relatively wide variety. The synthetic resins which may be used are the phenolic base resins, the vinyl acetate or chloride resins, the cellulose acetate or nitrate resins, and the polyvinyl alcohol resins, to mention only a few. Likewise, the hydrocarbon resins such as terpene polymers, styrene polymers, etc., and the coal tar distillate resins such as the coumarone-indene resins, including polycoumarone, polyindene and copolymers of coumarone with indene and their homologs, may also serve effectively. A typical composition which may be employed for the adhesive coating is as follows:

|                                                   | Per cent |
|---------------------------------------------------|----------|
| 55 Paracoumarone-indene resin (in solution) ..... | 48.6     |
| Inert, transparent pigment .....                  | 1.6      |
| Dibutyl phthalate .....                           | 0.1      |
| Butyl Cellosolve (2-butoxy ethanol) .....         | 1.2      |
| Hydrocarbon solvent .....                         | 48.5     |
|                                                   | 100.0    |

Another adhesive composition which has been found to give excellent results is as follows:

|                                                | Per cent |
|------------------------------------------------|----------|
| Paracoumarone-indene resin (in solution) ..... | 80       |
| Ethyl cellulose .....                          | 20       |
|                                                | 100      |

After the solution of the resin has been applied over the layer D, the solvent evaporates leaving behind a residual dry layer R which is non-tacky and non-pressure sensitive. It is an important feature of our invention that the solvent selected

to form the resin solution should be quick-drying in order to render the decalcomania sheets readily stackable and printable during this intermediate stage of their production. We have found that by selecting a solvent of appropriate volatility or by blending several solvents to obtain the desired degree of volatility, we can achieve a workable dry condition of the layer R in a relatively short time, e. g. 15 to 20 minutes or less. Thereafter, the sheets may be stacked one on top of the other 10 while awaiting application of the design layers, thus eliminating the necessity of space-consuming drying and separating racks.

Over the layer R is then printed or screened an activating layer A whose active constituent is a 15 plasticizer or a mixture of plasticizers having an affinity for and capable of acting upon or reacting with the resinous component of the adhesive layer R to impart to the latter the desired degree of tack and pressure sensitivity. The activating 20 layer is preferably in the form of a solution, such as a nitro-cellulose lacquer, comprising a suitable solvent and a sufficient amount of an appropriate plasticizer to migrate or diffuse from the activating 25 layer A to the adhesive layer R. Many types of plasticizers may be employed including the phthalate esters, such as dibutyl phthalate and diphenyl phthalate; the carboxylic acid esters such as triacetin, butyl oleate, butyl acetyl ricinoleate, dibutyl sebacate, glyceryl sebacate, methyl 30 abietate, and triethylene glycol hexoate; the phosphate esters such as tributyl phosphate, tricresyl phosphate, and diphenyl mono-(o-xenyl) phosphate, etc. In general, however, the selection 35 and the formulation of the plasticizing components of the activating layer A are correlated with the type of resin in the adhesive layer R to obtain the desired degree of pressure sensitivity.

We have obtained excellent results by employing 40 for the activating layer A a normal outdoor lacquer containing glyceryl sebacate as a plasticizer. Another and more specific formula which we have found to be suitable for use in the layer A, particularly when the first adhesive composition 45 specifically disclosed above is employed in the layer R, is as follows:

|                                     | Per cent |
|-------------------------------------|----------|
| Nitro-cellulose                     | 15.0     |
| Dibutyl phthalate                   | 1.4      |
| Castor oil                          | 21.0     |
| Butyl Cellosolve (2-butoxy ethanol) | 46.7     |
| Talc                                | 15.9     |
|                                     | <hr/>    |
|                                     | 100.0    |

The foregoing composition is particularly useful where a clear activating coat is desired. In instances where it may be desirable to employ an opaque activating layer to provide, for example, a white background for the subsequent color print layers, the following activating layer composition may be used:

|                                     | Per cent |
|-------------------------------------|----------|
| Nitro-cellulose                     | 12.8     |
| Titanium dioxide                    | 34.2     |
| Soybean oil                         | 6.8      |
| Dibutyl phthalate                   | 6.8      |
| Castor oil                          | 6.8      |
| Butyl Cellosolve (2-butoxy ethanol) | 17.1     |
| Butyl alcohol                       | 6.8      |
| Butyl acetate                       | 8.7      |
|                                     | <hr/>    |
|                                     | 100.0    |

As soon as the activating layer A, containing the plasticizer for the resin in the layer R, is

applied, the plasticizing components, comprising the castor oil and dibutyl phthalate of the first example or the soybean oil, dibutyl phthalate and castor oil of the second example, begin immediately to migrate or diffuse to the resinous layer. It has been observed that the plasticizer in the activating layer has a definite affinity for the resin in the adhesive layer and that migration occurs regardless of the relative positions of the two layers in the decalcomania provided, of course, that there is no sealing or isolating stratum interposed between the activating and adhesive layers which would prohibit the passage of the plasticizer. The plasticizer, reaching the adhesive layer in a relatively short time, imparts tacky and pressure sensitive properties to the resinous ingredient. The migration phenomenon of the plasticizer continues over a relatively long period of time, e. g. from 2 to 30 days, and the degree of pressure sensitivity in the adhesive layer R increases with the extent of migration. The solvent contained in the activating layer assists and initiates the migration of the plasticizer by preconditioning or penetrating the dry adhesive film ahead of the plasticizer and by providing, in effect, a softer and more receptive stratum for entry of the plasticizer.

With a given combination of resin in the layer R and plasticizer in the layer A, the degree of pressure sensitivity of the layer R may be controlled within specified limits dependent upon the particular use or intended application of the finished decalcomania. For example, if the final decalcomania is to be employed on a relatively smooth hard surface such as glass, only a moderate degree of pressure sensitivity in the layer R will be required, but if the decalcomania is to be applied to relatively rough or "difficult" surfaces, such as fruit skins or wood surfaces, a higher degree of pressure sensitivity will be desired. In the decalcomania comprising the present invention, accurate control over the degree of pressure sensitivity in the adhesive layer R may be exercised by varying the respective amounts of the resin in the layer R and of the plasticizer in the layer A. If, for example, the finished decalcomanias are to be applied to the rough, waxy outer surfaces of oranges, it may be desirable to employ for the activating layer A a "stepped-up" lacquer, i. e. a nitrocellulose lacquer to which has been added a greater than normal amount of plasticizer. For other uses, the normal plasticizer content of the lacquer may suffice. In addition, the ultimate degree of pressure sensitivity of the layer R may also be regulated by the resin content of the layer R and also by the relative thicknesses of the layers R and A.

After the activating layer A has dried to a non-tacky condition, the desired transfer design 60 layer P is applied thereover in any of the well-known manners, such as by printing, screening, or lithographing. Usually, the transfer design is a composite design formed by superimposing various colored layers until the desired final design is obtained, such various design printings being indicated by the single layer P in the several figures of the drawing. A protective outer coating C of clear lacquer may then be added where necessary or desirable to protect the 65 printed design during handling and storage of the decalcomanias. The colored inks employed in the application of the layer P are ordinarily special lacquer base inks and, therefore, contain substantial quantities of plasticizing compounds 70 which will also migrate or diffuse through the

activating layer A into the adhesive layer R and thereby assist in converting the resinous layer to a tacky, pressure sensitive condition. It is to be noted, however, that although the resinous adhesive layer R becomes tacky and pressure sensitive, the later lacquer layers, including the activating layer A and the design layers P, are not in any way prevented from becoming non-tacky and from remaining in a tough flexible state.

A decalcomania produced in the manner above-described and according to the layer arrangement shown in Fig. 1 is applied in much the same manner as the conventional "slip-off" transfer. The decalcomania is first dipped in water or the backing B is otherwise wetted with water to 15 soften the gummy layer D. When the water soluble layer D has dissolved sufficiently, the adhesive layer R and the layers superimposed thereon are released, and the backing sheet B is slid off exposing the pressure sensitive layer R. The 20 decalcomania is then applied by pressing the tacky layer R into contact with the surface to be decorated. The pressure sensitivity of the layer R provides a firm initial bonding action which is 25 highly satisfactory in causing the design to adhere readily to all types of "difficult" surfaces. However, in contrast with the known types of pressure sensitive decalcomanias, the volatile components in the pressure sensitive layer R evaporate with the passage of time, and by 30 gradual drying and polymerization of the resinous constituents, the layer R develops into a permanent, tough, strong, scratch resistant bond with the decorated surface. Thus, it will be seen that the initial pressure sensitive bond afforded by the tacky layer R is converted by a chemical 35 bonding reaction, after the lapse of time, to a permanent, hard, flexible bond with the underlying surface.

In Fig. 2 a slightly modified form of decalcomania embodying the migration principle of the present invention is illustrated. The backing or carrier sheet B coated with the water soluble adhesive layer D and the resinous adhesive layer R are the same as in the transfer 40 illustrated in Fig. 1. However, in this embodiment of the invention the color printing ink layer P is applied directly over the adhesive layer R after the latter has dried. The activating layer A is applied directly on the design layer P and serves also to protect the printed design thereby eliminating the necessity for a separate 45 protective coating C. In this form of the invention the plasticizing oils in the activating layer A migrate or diffuse downwardly through the printed design layer P, which does not impede or prevent the desired migratory action, and pass in combination with the plasticizer contained in the inks of the layer P into the adhesive layer R. A decalcomania of the type of 50 Fig. 2 may be applied to a surface in the same manner as described above in connection with Fig. 1 and with the same satisfactory results.

A different type of decalcomania embodying the migration principle is illustrated in Fig. 3. This form of transfer may be characterized as a "reverse" type of decalcomania in that the color printing layer P is applied directly over the water soluble adhesive layer D carried by the backing sheet B, and the activating layer A and the 55 resinous adhesive layer R are applied in the stated order over the printing layer P. Migration of the plasticizing oils from the layers A and P then occurs in an upward direction into the adhesive layer R imparting tack and pres-

sure sensitivity to the latter. In this form of the invention a water soluble sealer coat S, such as a water soluble glue, gum acacia, dextrine, etc., is applied over the layer R to permit the decalcomania to be readily handled and stored. In the application of this type of decalcomania, the transfer is wetted with water on both sides thereby dissolving the layer D to permit the transfer to be removed from the backing sheet B and also dissolving the top layer S to expose the tacky, pressure sensitive layer R by means of which the transfer is caused to adhere initially to the desired surface in the manner hereinbefore described.

Figs. 4 and 5 constitute modified forms of the decalcomania of the present invention in which no special activating layer is employed and where tack of a relatively low degree is desired. In the embodiment shown in Fig. 4 the color printing layer P is applied directly over the resinous adhesive layer R and the natural plasticizing components present in the inks employed to form the layer P migrate downwardly into the layer R imparting the desired tack and pressure sensitivity thereto. A protective coating C is provided to prevent injury to the printed design P.

In Fig. 5, a "reverse" type decalcomania is illustrated in which no special activating layer is used. The color print P is applied directly to the dextrine coating D of the backing sheet B, and the adhesive layer R is superimposed on the layer P. The plasticizing components in the inks of the layer P migrate upwardly to the layer R converting the latter to a tacky, pressure sensitive state. As in the "reverse" type decalcomania described in connection with Fig. 3, the form of the invention illustrated in Fig. 5 also requires a final water soluble sealer coating S for protecting the pressure sensitive layer R until it is desired to use the transfer. The decalcomania shown in Figs. 4 and 5 are used in the same manner described above in connection with Figs. 1 and 3, respectively, and the adhesive layers, after lapse of time, form relatively dry, tough, flexible bonds.

Although several forms of decalcomanias with the component layers thereof in various arrangements have been disclosed in Figs. 1 to 5, inclusive, of the drawing, and several specific examples as to the constituent elements of the adhesive layer and the activating layer have been given, it is apparent that modifications in the adaptation of the migration principle may be resorted to without departing from the scope of the invention as defined in the appended claims.

We claim:

1. A method of forming a pressure sensitive decalcomania which comprises separately applying in predetermined sequence over one side of a releasable backing an adhesive material comprising a solution of a thermoplastic resin in a volatile solvent and an activating material comprising a plasticizer-containing lacquer, permitting the first-applied material to dry to a normally non-tacky and non-pressure sensitive state prior to application of the other of said materials, thereafter permitting said other material to dry to a normally non-tacky and non-pressure sensitive state whereby to form separate and initially non-pressure sensitive resinous and lacquer layers disposed in superimposed relation one above the other on said backing, said lacquer layer containing a sufficient quantity of a

readily migratable plasticizer to render said resinous layer tacky and pressure sensitive, and allowing said plasticizer to migrate to the resinous layer thereby converting the latter to a tacky and pressure sensitive condition.

2. The method of claim 1 further characterized in that said resin comprises a coumarone-indene resin.

3. A method of forming a pressure sensitive decalcomania having a water permeable backing with a water soluble film thereon which comprises applying over said film a solution comprising a thermoplastic resin in a volatile solvent, permitting said solution to dry to form a normally non-tacky and non-pressure sensitive resinous layer, subsequently applying thereover a lacquer containing a sufficient quantity of a readily migratable plasticizer to render said resinous layer tacky and pressure sensitive, and allowing said plasticizer to migrate to the resinous layer thereby converting the latter to a tacky and pressure sensitive condition.

4. A method of forming a pressure sensitive decalcomania having a water permeable backing with a water soluble film thereon which comprises applying over said film a solution comprising a thermoplastic resin in a volatile solvent, permitting said solution to dry to form a normally non-tacky and non-pressure sensitive resinous layer, subsequently applying directly thereover a plasticizer-containing lacquer, permitting said lacquer to dry to form a non-pressure sensitive lacquer layer, thereafter applying a transfer design directly over said lacquer layer, said lacquer layer containing a sufficient quantity of a readily migratable plasticizer to render said resinous layer tacky and pressure sensitive, and allowing said plasticizer to migrate to the resinous layer thereby converting the latter to a tacky and pressure sensitive condition.

5. A method of forming a pressure sensitive decalcomania having a water permeable backing with a water soluble film thereon which comprises applying over said film a solution comprising a thermoplastic resin in a volatile solvent, permitting said solution to dry to form a normally non-tacky and non-pressure sensitive resinous layer, applying directly thereover a transfer design film, permitting the latter film to dry, subsequently applying directly over the design film a lacquer containing a sufficient quantity of a readily migratable plasticizer to render said resinous layer tacky and pressure sensitive, and allowing said plasticizer to migrate through said transfer design film to said resinous layer and thereby convert the latter to a tacky pressure sensitive condition.

6. A method of forming a pressure sensitive decalcomania having a water permeable backing with a water soluble film thereon which comprises applying a transfer design over said film, applying a plasticizer-containing lacquer layer directly over said design, applying directly over said lacquer layer a solution comprising a thermoplastic resin in a volatile solvent, permitting said solution to dry to form a normally non-tacky and non-pressure sensitive resinous layer, said lacquer layer containing a sufficient quantity of a readily migratable plasticizer to render said resinous layer tacky and pressure sensitive, and allowing said plasticizer to migrate to the resinous layer thereby converting the latter to a tacky and pressure sensitive condition.

7. A method of forming a pressure sensitive

decalcomania having a water permeable backing with a water soluble film thereon which comprises applying over said film a solution comprising a thermoplastic resin in a volatile solvent, permitting said solution to dry to form a normally non-tacky and non-pressure sensitive resinous layer, applying directly thereover a transfer design layer comprising a lacquer containing a sufficient quantity of a readily migratable plasticizer to render said resinous layer tacky and pressure sensitive, and allowing said plasticizer to migrate from said design layer to said resinous layer and thereby convert the latter to a tacky pressure sensitive condition.

15 8. A method of forming a pressure sensitive decalcomania having a water permeable backing with a water soluble film thereon which comprises applying a transfer design over said film, subsequently applying directly over said transfer design a solution comprising a thermoplastic resin in a volatile solvent, thereafter permitting said solution to dry to form a normally non-tacky and non-pressure sensitive resinous layer, said transfer design comprising a lacquer containing a sufficient quantity of a readily migratable plasticizer to render said resinous layer tacky and pressure sensitive, and allowing said plasticizer to migrate to said resinous layer and thereby convert the latter to a tacky pressure sensitive condition.

30 9. A decalcomania of the pressure sensitive type prepared in accordance with the method of claim 1.

10. A decalcomania of the pressure sensitive type prepared in accordance with the method of claim 2.

11. A decalcomania of the pressure sensitive type prepared in accordance with the method of claim 3.

40 12. A decalcomania of the pressure sensitive type prepared in accordance with the method of claim 4.

13. A decalcomania of the pressure sensitive type prepared in accordance with the method of claim 5.

14. A decalcomania of the pressure sensitive type prepared in accordance with the method of claim 6.

50 15. A decalcomania of the pressure sensitive type prepared in accordance with the method of claim 7.

16. A decalcomania of the pressure sensitive type prepared in accordance with the method of claim 8.

55 ALFRED F. GRUPP.  
HARRY C. RATHKE.  
ELWOOD S. TALAN.  
ELMORE WATTS.

#### REFERENCES CITED

The following references are of record in the file of this patent:

#### UNITED STATES PATENTS

| 65 | Number    | Name            | Date           |
|----|-----------|-----------------|----------------|
|    | 1,627,407 | Reese           | May 3, 1927    |
|    | 1,780,021 | Laws            | Oct. 28, 1930  |
|    | 1,826,228 | Tull            | Oct. 6, 1931   |
|    | 1,104,025 | Davis           | Jan. 4, 1938   |
| 70 | 2,271,413 | Braverman       | Jan. 27, 1942  |
|    | 2,359,185 | Wysong          | Sept. 26, 1944 |
|    | 2,409,564 | Heinecke et al. | Oct. 15, 1946  |
|    | 2,453,052 | Van Etten       | Nov. 2, 1948   |